

## UNITED STATES PATENT OFFICE

2,132,930

## VISCOSE SPINNING SOLUTION

Rudolph S. Bley, Elizabethton, Tenn., assignor to  
 North American Rayon Corporation, New York,  
 N. Y., a corporation of Delaware

No Drawing. Application December 2, 1937,  
 Serial No. 177,825

12 Claims. (Cl. 106—40)

In the manufacture of cellulosic products, such as filaments, threads, and the like, a viscose solution is continuously extruded through the minute orifices of a spinneret into a coagulating or setting bath (spin bath). However, since the introduction of the viscose process great troubles have been and are still experienced as far as continuous spinning is concerned due to impurities, such as, for example, precipitated cellulose particles, sulphur and resin particles, zinc compounds, etc., present in either the viscose solution or the spin bath. These impurities gradually contaminate the spinnerets, clog and reduce the widths of the spinneret holes with the result that filaments of uneven thickness are obtained. If the contamination of the spinnerets and the clogging of their holes proceeds the individual filaments start to tear and occasion interruption of the spinning process.

By experimentation, I have found that the contamination of spinnerets and the clogging of spinneret holes may be overcome by spinning viscose solutions in the presence of cation-active compounds, these compounds being produced by condensing a halogenated petroleum or a halogenated petroleum constituent containing at least one hydrocarbon having a chain of eight or more carbon atoms with an organic sulphide, selected from the group consisting of dialkyl sulphides, diaryl sulphides and alkyl-aryl sulphides under substantially anhydrous conditions.

Petroleum consists of complex mixtures of hydrocarbons concerning the chemical nature of which there is very little information, although there are indications that all of these materials contain members of the methane series, the polymethylene series and the benzene series of hydrocarbons. The difference between petroleums of various sources resides in the proportions of the different types of hydrocarbons and in the chemical nature and amounts of their impurities. Pennsylvania oil, for example, contains a large proportion of methane hydrocarbons and practically no impurities of sulphur or nitrogen compounds. About thirty hydrocarbons have been isolated and identified with certainty. Distillation is the principal method in separating petroleum into useful components. The distilled fractions from crude petroleum are casinghead gasoline, gasoline, kerosene, gas oil and lighter lubricating oils (" neutrals"). The residues from such distillation supply most of the lubricating oils ("bright stock"), petrolatum in pasty or liquid form and either paraffin wax or petroleum pitch,

depending upon the nature of the crude petroleum. Kerosene is any mixture of hydrocarbons which is not volatile enough for use in explosion motors. Cracked gasolines are rich in olefins and diolefins. Paraffin wax was originally obtained from tars from the distillation of wood, peat, and lignite, but is now obtained from petroleum, and especially from Pennsylvania paraffin-base oils. Little information is available about the composition of paraffin waxes except that it consists mainly of higher alkanes and only small amounts of the normal compounds. Petrolatum (vaseline) is a pasty mixture of hydrocarbons similar to paraffin while liquid petrolatum is a high boiling petroleum distillate. Ozokerite is a natural paraffin wax originating in Galicia; in bleached form it is termed "ceresin". All of these petroleum hydrocarbons may be halogenated in conventional manner in the presence or absence of catalysts to form halogenated hydrocarbon mixtures adapted to be condensed with the tertiary bases and organic sulphides, set forth above. The materials, i. e., crude petroleums, gasolines, kerosenes, lubricating oils, pasty petrolatums, liquid petrolatums and paraffin waxes, to be halogenated may first be dissolved in carbon tetrachloride, etc., and subsequently chlorine, bromine, etc., in gaseous form introduced therein until the heat of reaction abates. Halogenated compounds, containing about 25 to 40% of halogen may be obtained in this manner. However, upon prolonging the introduction of halogens, compounds may be obtained containing up to about 75% of a halogen, and it is to be noted that the boiling or fusing points of the raw materials are either lowered or raised by halogenation. Hydrochloric acid, hydrobromic acid, etc., formed during this reaction must be removed, preferably by neutralization. Catalysts, such as iron, etc., may be added to the mixtures to accelerate halogenation. Halogenation will also proceed more rapidly by carrying out the reaction under the influence of ultra-violet rays. The halogenation may also be performed in accordance with processes disclosed, for example, in U. S. Patent #989,225 to Blakeman of April 11, 1911; U. S. Patent #1,246,810 to Ellis of November 13, 1917; U. S. Patent #1,432,761 to Kock of October 24, 1922; etc. Chlorinated paraffin wax, sold under the trade name of "Chlorafin" is a very suitable raw material for my process.

Organic sulphides capable of being condensed with the halogenated, hydrocarbonaceous materials set forth above are dialkyl sulphides, diaryl

sulphides and alkyl-aryl sulphides, having the following structure:

5



in which  $R_1$  and  $R_2$  represent monovalent aliphatic (alkyl) or aromatic (aryl) radicals. Examples of such organic sulphides are dimethyl sulphide, diethyl sulphide, methyl-ethyl sulphide, methyl-propyl sulphide, dibutyl sulphide, methyl-benzyl sulphide, propyl-ethyl sulphide, dibenzyl sulphide, diphenyl sulphide, etc.

Thus, by condensing an organic sulphide with 15 a halogenated, hydrocarbonaceous material of the aforementioned group, sulphonium halides are obtained, having the structure:

20



in which  $P$  represents a petroleum hydrocarbon chain. If  $P$  is a chain containing eight or more carbon atoms the sulphonium halide becomes 25 cation-active and an incrustation inhibitor. Cation-active compounds are surface-active compounds which carry in the cation a hydrocarbon chain having eight or more carbon atoms. They 30 are particularly advantageous because they may be used in neutral (salt), alkaline and acidic aqueous solutions, and also in hard water. In contradistinction to cation-active compounds, anion-active compounds are surface-active compounds which carry in the anion a more or less 35 extended hydrocarbon chain (fat chain). They flocculate in neutral (salt), alkaline and acidic aqueous solutions, and also in hard water. Common soaps, sulphonated oils, salts of sulphonated fatty acids, etc., are examples of anion-active 40 compounds, and they are unable to prevent the incrustation of spinnerets and spinneret holes. These incrustation inhibitors are prepared by 45 heating a halogenated hydrocarbonaceous material selected from the group consisting of crude petroleums, gasolines, kerosenes, lubricating oils, pasty petrolatums, liquid petrolatums and paraffin waxes with an organic sulphide at a moderate 50 temperature—preferably under reflux—until condensation is completed. Before heating the two 55 components they may be dissolved in a suitable, inert solvent, such as, for example, benzene, ether, toluene, etc., i. e., in solvents which are incapable of chemically reacting with the compounds to be condensed. The inert solvent may 60 subsequently be removed from the condensation products by distillation, and the unreacted sulphide may be separated from the condensation products by distillation, extraction, etc. The crude incrustation inhibitors may contain a number 65 of different condensation products which need not be separated from each other. In other words, the crude condensation products (incrustation inhibitors) containing cation-active and cation-inactive constituents may, for reasons 70 of economy, be added without further purification to viscose solutions or spin baths (setting baths). Although these cation-active halides, i. e., bromides, chlorides, iodides and fluorides, may form sulphonium bases in viscose solutions and sulphonium salts in acid spin baths, they retain 75 their surface-activity and, thus, their property of preventing incrustation. If very small amounts of these condensation products are added to viscose solutions or spin baths the physical characteristics, such as strength, plasticity, lustre, etc.,

of regenerated cellulose produced therefrom or therein, respectively, remain practically unaltered. Upon increasing the amount of incrustation inhibitor in a given viscose solution or spin bath, the regenerated cellulose produced therefrom or therein, respectively, may alter its physical characteristics, i. e., it may acquire a soft lustre, become more plastic, lose part of its original strength, etc. For such reasons, the amounts of such compounds to be added to viscose solutions or spin baths control the physical properties of the finished cellulosic products. In other words, these additions are critical and their amounts must be predetermined by experimentation. Additions of about 0.3 to 1.0 gram per liter 10 of viscose or spin bath are insufficient to substantially alter the physical characteristics of regenerated cellulose although they allow continuous spinning for long periods of time.

Although these cation-active sulphonium compounds 20 improve the spinning properties of any conventional viscose solution or any spin bath known in the art, I have found that they are especially valuable additions to zinc-bearing baths which tend to interrupt spinning, i. e., spin baths 25 containing zinc compounds, such as, for example, zinc sulphate.

#### Example I

Ethyl-methyl sulphide is condensed with a 30 halogenated, hydrocarbonaceous material selected from the group consisting of crude petroleums, kerosenes, gasolines, lubricating oils, pasty petrolatums, liquid petrolatums and paraffin waxes by heating under reflux until condensation is 35 completed. About 0.4 to 1.0 gram of the condensation products are added to one liter of a viscose solution of conventional cellulose content and maturity. This solution is then spun into a conventional, acid spin bath, such as, for example, a glucose bath, a magnesium-zinc bath, 40 etc. The spinnerets and spinneret holes remain clean on prolonged spinning in comparison with the spin bath free from cation-active compounds. Any dialkyl sulphide, diaryl sulphide or alkyl-aryl sulphide may be used in the condensation, 45 which may be carried out at any temperature at which the two reactants and the sulphonium halide remain stable.

#### Example II

An alkyl-aryl sulphide, a dialkyl sulphide or a diaryl sulphide, such as, for example, dibenzyl sulphide is condensed with a halogenated paraffin wax in the presence of an inert solvent, such as, 55 for example, benzene, etc., under substantially anhydrous conditions. A conventional viscose solution is extruded through fine orifices of a spinneret of a precious metal into an acid spin bath, this bath containing sulphuric acid, sodium sulphate, ammonium sulphate and zinc sulphate plus about 0.05% by weight of a cation-active substance set forth above. Spinning irregularities and difficulties are substantially overcome while without this inhibitor spinning is interrupted after a very short period of time. These 65 inhibitors are especially suitable for continuous spinning processes using sulphuric acid-zinc sulphate baths. These sulphides may be condensed with any halogenated, hydrocarbonaceous material of the group set forth above.

#### Example III

Cation-active condensation products are added to both the viscose solutions and the spin baths 75

to allow continuous formation of lustrous or soft-lustre viscose products.

Although these examples will serve to illustrate the present invention, I do not wish to be limited to the inhibitors and concentration thereof recited therein, since I may use any cation-active sulphonium compound of the group set forth above and vary the physical characteristics of regenerated cellulose by varying their amounts in viscose solutions and/or spin baths, provided these inhibitors are sufficiently soluble in viscose solutions and/or spin baths to furnish cations therein.

Modifications of my invention will readily be recognized by those skilled in the art, and I desire to include all such modifications and variations coming within the scope of the appended claims.

I claim:

1. A spinning solution for the manufacture of artificial products comprising a viscose solution and a cation-active condensation product of a halogenated hydrocarbonaceous material selected from the group consisting of halogenated crude petroleums, halogenated gasolines, halogenated kerosenes, halogenated lubricating oils, halogenated pasty petrolatums, halogenated liquid petrolatums and halogenated paraffin waxes and an organic sulphide selected from the group consisting of dialkyl sulphides, alkyl-aryl sulphides and diaryl sulphides, said condensation product being sufficiently soluble in said viscose solution to become cation-active therein.

2. A spinning solution for the manufacture of artificial products comprising a viscose solution and a cation-active condensation product of a halogenated paraffin wax and ethyl-methyl sulphide.

3. A spinning solution for the manufacture of artificial products comprising one liter of a viscose solution and about 0.4 to 1.0 gram of a cation-active condensation product of a halogenated hydrocarbonaceous material selected from the group consisting of halogenated crude petroleums, halogenated gasolines, halogenated kerosenes, halogenated lubricating oils, halogenated pasty petrolatums, halogenated liquid petrolatums and halogenated paraffin waxes and an organic sulphide selected from the group consisting of dialkyl sulphides, alkyl-aryl sulphides and diaryl sulphides, said condensation product being sufficiently soluble in said viscose solution to become cation-active therein.

4. A spinning solution for the manufacture of artificial products comprising one liter of a viscose solution and about 0.4 to 1.0 gram of a

cation-active condensation product of a halogenated paraffin wax and ethyl-methyl sulphide.

5. A soft-lustre regenerated cellulose containing a finely divided cation-active condensation product of a halogenated hydrocarbonaceous material selected from the group consisting of halogenated crude petroleums, halogenated gasolines, halogenated kerosenes, halogenated lubricating oils, halogenated pasty petrolatums, halogenated liquid petrolatums and halogenated paraffin waxes and an organic sulphide selected from the group consisting of dialkyl sulphides, alkyl-aryl sulphides and diaryl sulphides in a sufficient amount to diminish the lustre thereof.

6. A soft-lustre regenerated cellulose containing a finely divided cation-active condensation product of a halogenated paraffin wax and ethyl-methyl sulphide in a sufficient amount to diminish the lustre thereof.

7. A spinning solution for the manufacture of artificial products comprising a viscose solution and a cation-active condensation product of a chlorinated paraffin wax and ethyl-methyl sulphide.

8. A spinning solution for the manufacture of artificial products comprising a viscose solution and a cation-active condensation product of a chlorinated paraffin wax and a dialkyl sulphide, said condensation product being sufficiently soluble in said viscose solution to become cation-active therein.

9. A spinning solution for the manufacture of artificial products comprising one liter of a viscose solution and about 0.4 to 1.0 gram of a cation-active condensation product of a chlorinated paraffin wax and ethyl-methyl sulphide.

10. A spinning solution for the manufacture of artificial products comprising one liter of a viscose solution and about 0.4 to 1.0 gram of a cation-active condensation product of a chlorinated paraffin wax and a dialkyl sulphide, said condensation product being sufficiently soluble in said viscose solution to become cation-active therein.

11. A soft-lustre regenerated cellulose containing a finely divided cation-active condensation product of a chlorinated paraffin wax and ethyl-methyl sulphide in a sufficient amount to diminish the lustre thereof.

12. A soft-lustre regenerated cellulose containing a finely divided cation-active condensation product of a chlorinated paraffin wax and a dialkyl sulphide in a sufficient amount to diminish the lustre thereof.

RUDOLPH S. BLEY. 55